

Jan. 14, 1941.

T. L. MADDOCK

2,228,281

TRANSFERABLE MATERIAL FOR SURFACE SHADING SHEETS

Original Filed April 26, 1938



INVENTOR.  
Theodore L. Maddock,  
BY  
T. Baker, Galnick & Newark  
ATTORNEYS.

## UNITED STATES PATENT OFFICE

2,228,281

TRANSFERABLE MATERIAL FOR SURFACE  
SHADING SHEETSTheodore L. Maddock, Cleveland, Ohio, assignor  
to Fine Art Manufacturing Company, Cleve-  
land, Ohio, a corporation of OhioOriginal application April 26, 1938, Serial No.  
204,343. Divided and this application Novem-  
ber 23, 1938, Serial No. 242,047

2 Claims. (Cl. 134—28)

My prior application, Serial No. 204,343, filed April 26, 1938, shows and describes a Method and means for shading surfaces, comprising causing isolated areas of transferable material regularly arranged on a thin, tough, flexible, transparent sheet of thermo-plastic material to be transferred by pressure on the back of such sheet to an underlying figure to be shaded.

While the parent application referred to is now concerned only with the method of carrying out the operation, it describes the articles used in the performing of such method, comprising a thin transparent cellulose sheet and a peculiar transferable material affixed thereto. The present application, which is a division of the parent application referred to, is concerned with the transferable material adapted to be affixed to the transparent cellulose sheet.

The application mentioned describes a sheet of Cellophane, preferably laminated in different directions to prevent curling, and a black transferable substance adapted to be applied to such sheet by a pressing operation, and sets out in detail the composition of the transferable substance. However, I have found that a unitary sheet of thermo-plastic material comprising a film of cellulose acetate similar to the film used for photographic negatives, is preferable to a laminated Cellophane sheet. Such cellulose film with the transferable material applied thereto in regular isolated areas forms the subject matter of an application of mine Serial No. 242,011, filed November 23, 1938, which is a continuation in part of said application No. 204,343.

It will be understood that the sheet employed is tough, flexible and transparent, and by causing proper transferable material to adhere to it, I may use the sheet as an impression member, placing it over the drawing or other matter to be shaded, then by pressure of the artist's pencil on top of the sheet, transfer shaded material to the underlying surface.

Not only has there been difficulty in securing a material which will adhere to the sheet with sufficient rigidity so that it will not be inadvertently displaced or rubbed off in storage, but will not adhere so firmly as to prevent transfer, and which will not deteriorate or become hard or glossy with time. After considerable experimenting, I have discovered a composition which may be handled like printers' ink and applied by a printing operation to the cellulose or Cellophane film, and which will not spread after being printed

thereon, and will become comparatively dry and effectively retain its position on the sheet, but which may be transferred to the underlying sheet by pressure on top of the film.

The transferable material employed on ordinary carbon sheets used in typewriting, etc., will not adhere to Cellophane or to other cellulose acetate film. On the other hand, the inks which have been developed for printing on Celluloid, Cellophane and other synthetic sheets, will not offset.

I have found that I can accomplish excellent results by employing the following composition, which forms the subject matter of this application, as specified in the claims, namely:

|                 | Parts |
|-----------------|-------|
| Ester gum       | 4     |
| Linseed varnish | 8     |
| Carbon black    | 4     |
| Orange toner    | 2     |
| Carnauba wax    | 1     |
|                 | 20    |

The above materials are ground together to make a composition of consistency similar to ordinary printers' ink. This material is placed in the fountain of a suitable press, and an imprint is made on the film by an engraved roller carrying whatever figure is to be imprinted, as, for instance, the dots or parallel lines. After the imprinting substance has been allowed to dry, the cellulose sheet carrying the same is secured face down on the protection sheet, and the product is ready for use.

The drawing is a diagram illustrating the composition, the primary ingredients being indicated by full lines, and an optional, though preferred ingredient indicated by broken lines.

I claim:

1. A composition of substantially four parts ester gum, eight parts of linseed varnish, four parts of carbon black and one part of carnauba wax of a consistency enabling it to adhere to a sheet of transparent material of the group containing Cellophane and cellulose acetate, and be transferable therefrom at ordinary temperature by pressure on the back of the sheet.

2. A composition adapted for printing on a sheet of cellulose acetate, to adhere thereto but be transferable therefrom at ordinary temperature by pressure, comprising substantially four parts ester gum, eight parts linseed varnish, four parts carbon black, one part carnauba wax and two parts orange toner.

THEODORE L. MADDOCK.